

## UNITED STATES PATENT OFFICE

2,683,107

## MANUFACTURE OF PITCH

Leslie Harrisville Juel, Arlington Heights, Ill., assignor to Great Lakes Carbon Corporation, New York, N. Y., a corporation of Delaware

No Drawing. Application October 5, 1951,  
Serial No. 250,015

5 Claims. (Cl. 196—14.1)

1

This invention relates to a process for manufacturing carbonaceous compositions useful in the manufacture of carbon and graphite electrodes. More particularly, the invention relates to a process of manufacturing binders and impregnating agents from coal-derived bitumens.

This application is a continuation-in-part of my co-pending application Ser. No. 106,329, filed July 22, 1949 for Manufacture of Pitch, now abandoned.

In the usual practice of manufacturing graphite electrodes which are currently employed in electrothermal and electrometallurgical high temperature processes a carbonaceous aggregate, preferably petroleum coke which has been calcined to less than 1% volatile matter, is admixed with suitable amounts of a binder to form a composition which is extruded or molded. The resulting body is then baked and graphitized. In order to increase the strength and apparent density of the baked or graphitized carbons they are often impregnated under vacuum with liquid carbonaceous materials which are subsequently carbonized.

The most commonly used binder and impregnant at the present time is pitch derived from coal tar. This pitch is a heterogeneous mixture of complex hydrocarbons which may be broadly classified into about four fractions; namely, a fraction insoluble in organic solvents and insoluble in the pitch itself even when the latter is heated to temperatures up to about 400° C.; a fraction which is soluble in the coal tar (particularly when heated) but insoluble in low-boiling aromatic solvents such as benzene; a fraction which is soluble in benzene but insoluble in paraffinic hydrocarbons such as solvent naphtha, and a fraction which is soluble in benzene and in solvent naphtha and low boiling aliphatic compounds. It is known that certain fractions of coal tar or pitch derived therefrom are particularly suitable as binders for carbon particles in the manufacture of carbon and graphite electrodes. Others have stated that the benzene-insoluble fraction exhibits poor binding or adhesive qualities with respect to the carbon aggregate. The solvent naphtha-soluble fraction exhibits some binding characteristics but is somewhat objectionable in that it produces a low coke residue in the electrode baking operation. It has been pointed out that the benzene-soluble fraction constitutes the most advantageous fraction of coal tar or coal tar pitch for a binder for the carbon particles in that it combines the advantages of high coke residue with good adhesion to the particles.

Several investigators have proposed to prepare a carbonaceous binder for carbon particles suitable in the manufacture of carbon electrodes from coal tar and pitches by employing a se-

2

quence of solvent extraction operations whereby the benzene-soluble fraction is isolated substantially free from the tar-insoluble, benzene-insoluble and solvent naphtha-soluble fractions. This is both time consuming and economically prohibitive from a commercial standpoint. It has also been proposed to prepare a carbonaceous binder for carbon particles by distilling coal tar or coal tar pitch, either at atmospheric pressure or in a vacuum, in order to obtain a comparatively high boiling distillate which is substantially soluble in benzene but which also contains substantial quantities of the undesirable solvent naphtha-soluble components which produce a low coke residue. The latter type of operation further suffers from the fact that up to 40% by weight of the original pitch or tar so distilled remains in the still as pitch coke and the yields of binder so produced are consequently not very high.

It is an object of this invention to provide a carbonaceous composition suitable as a binder for carbon aggregate in the manufacture of carbon electrodes, particularly of the graphite type.

It is a further object of the invention to provide a process for the manufacture of carbonaceous binders and impregnating agents which are substantially free from matter undissolvable therein and which contain substantial quantities of benzene-insoluble components having a high coke residue.

It is a further object of the invention to provide a carbonaceous material having improved coking characteristics which render it particularly suitable for the manufacture of graphite electrodes.

It is a further object of the invention to provide graphite electrodes having lower electrical resistivities than graphite electrodes produced with the conventional type of coal tar pitch binders.

The above objects as well as others which will become apparent upon a complete understanding of the invention are accomplished by removing from coal-derived bitumen substantially all of the material contained therein which is insoluble and undissolvable in the bitumen even at elevated temperatures, such as up to 400° C. According to my invention, the removal of the aforesaid objectionable material from the coal-derived bitumen is accomplished without substantially affecting or reducing the benzene-insoluble or benzene-soluble content of the bitumen. The treated bitumen is then heated, if necessary, under controlled conditions to raise its melting point and to increase the benzene-insoluble content without causing formation of material which is insoluble and undissolvable in the treated bitumen.

In a broad embodiment the present invention

comprises removing from a high boiling liquefiable coal-derived bitumen matter which is insoluble and undissolvable therein even when the bitumen is heated for a time insufficient to cause substantial coking thereof. This is accomplished in a manner such that the resulting product will be substantially free from an insoluble phase while retaining substantial amounts of benzene-insoluble matter which either was originally present in the material or was formed during the treatments described herein. I have found that the presence of the aforementioned undissolvable material in the bitumens which I employ has several disadvantages when such compositions are used as a binder or impregnating agent for carbon particles in the manufacture of graphite electrodes. The presence of such material in electrode binders and impregnants is believed to prevent the maximum and desirable degree of penetration or impregnation of the carbon particles by the more fluid components of the binder. Furthermore, the presence of this insoluble matter in the binder is detrimental to the formation of binder coke having a highly desirable structure during the electrode baking operation.

The removal of the aforesaid undissolvable material from the high boiling liquefiable coal-derived bitumen compositions may be conducted advantageously by filtration and centrifugation processes, which will be further herein described, as contrasted with distillation techniques either at atmospheric pressure or at subatmospheric pressures. As previously explained herein, the distillation processes heretofore employed to produce liquid or liquefiable carbonaceous binders and impregnants from coal tar or pitch produce materials which are substantially free from benzene-insoluble material. One of the important characteristics of the compositions produced in accordance with the present invention is the retention therein of a substantial amount of benzene-insoluble material which nevertheless is soluble or dissolvable in the composition itself, and which will produce a high coke residue in the carbon electrode during baking.

The high boiling liquefiable bitumens with which this invention is particularly concerned include coal derivatives such as retort and coke oven tars and pitches, water gas tars and pitches, straight run or cracked tars, and certain high boiling overheads produced from coal gasification processes. Included in the term pitch are the so-called soft, medium, and hard pitches having a softening point of 75° to 125° C. Other materials which are adaptable to the process of this invention are certain tar and pitch distillates which contain substantial amounts of benzene-insoluble matter and material undissolvable in the distillate itself, hydrogenated coal and certain distillates therefrom; lignite, brown coal, and tars and pitches therefrom. It has also been found that thermally produced dispersions of coal in oil which may or may not be subsequently hydrogenated, and certain distillates therefrom are useful in practicing the invention. The bitumens should be essentially hydrocarbonaceous in nature and substantially free from oxygen-containing compounds and inorganic matter. For the sake of brevity and convenience, these and related compositions are generically referred to herein as high boiling, liquefiable coal-derived bitumens. The aforementioned materials, particularly in their crude state, are characterized by the presence of varying amounts of undissolvable matter which may be removed

by filtration, centrifugation and equivalent methods according to this invention as contrasted with distillation of such materials.

This invention does not contemplate the treatment of petroleum base materials such as heavy residues or petroleum tars and pitches. Such materials are deficient in aromatic, coke-producing constituents. While they are substantially free from material which is insoluble and undissolvable in the main portion of the material they are also grossly deficient in benzene-insoluble matter, the latter being an essential component in the novel compositions described herein.

I have found that the removal of substantially all of the aforementioned undissolvable material from the liquefiable coal-derived bitumens, while retaining therein a substantial amount of benzene-insoluble matter which is soluble in the liquefiable portion of the bitumen (especially upon application of heat), produces a material which is particularly suitable as a binder for carbon aggregate and as an impregnating agent for massive carbons in the manufacture of carbon and graphite electrodes.

In a preferred embodiment of the invention, coal tar which contains matter insoluble and undissolvable therein even when the tar is heated to 400° C., is heated to a temperature between about 150° and 400° C. and the liquefied material is filtered, preferably in conjunction with a small quantity of diatomaceous earth filter aid. Usually between about 0.5 and 6% by weight of filter aid will suffice. The liquid material is fed to a filtration apparatus, for example a plate and frame filter press wherein the filtration medium such as canvas or heat-resistant material contains a pre-coat of filter aid of the diatomaceous earth type. The resulting filtrate is substantially free from the aforementioned undissolvable matter and will contain, after heat treatment, between about 15 and about 50% by weight of hydrocarbon material which is soluble or dissolvable in the filtrate itself but is insoluble in benzene and similar low boiling solvents. The filtrate may then be heated to temperatures preferably between about 400° and 525° C. and maintained in that temperature range until the material has a softening point of between about 35° and about 125° C. I have found that when the binders under consideration herein have a softening point above about 100° C. they are particularly desirable as binders for carbon aggregate in electrode manufacture.

In a further embodiment of the invention, coal tar or coal tar pitch is diluted with a high boiling aromatic solvent such as a coal tar distillate or highly aromatic petroleum fractions having a boiling range of about 250° to 350° C. Generally speaking, any aromatic solvent having a boiling point or boiling range between about 200° and about 400° C. may be employed provided that the major (liquefiable) portion of the coal bitumen is soluble therein. Paraffinic petroleum fractions such as so-called mineral or lubricating oils are not suitable for this operation. Such materials precipitate or leave undissolved the benzene-insoluble portion of the bitumen which is an essential element of my novel compositions. In adding an aromatic solvent to a commercial coal tar, a ratio of between about 20 and about 100 parts by weight of solvent to 100 parts by weight of tar has been found to be particularly satisfactory. For a coal tar pitch, a ratio of between about one and about five parts by weight of aromatic solvent to one part by weight of pitch is ad-

vantageous. Dilution of the liquefiable coal bitumen with solvents of the aforementioned type decreases the viscosity of the compositions and facilitates filtration. The extent of dilution should not exceed the point where substantial quantities of the desirable benzene-insoluble fraction of the coal bitumen will precipitate from the mixture. It is one of the main objects of the present invention to remove the bitumen-undissolvable matter from the bitumen while retaining substantial quantities of the benzene insoluble fraction in the final composition.

In the event that a solvent is employed in the filtration operation, the filtrate is preferably preliminarily heated to distill and recover the solvent followed by continued heating to produce a binder or impregnating agent having a melting point in the preferred range.

Removal of the objectionable undissolvable matter may also be accomplished by filtration on a rotary filter of the Oliver type, the latter containing a canvas or other suitable medium preferably pre-coated with a filter aid of the type previously mentioned herein as well as other suitable filter aids.

The undissolvable matter may also be removed by centrifugation operations, preferably subsequent to dilution of the coal bitumen in accordance with the above mentioned procedures.

In a further embodiment of the invention, I may add to the novel binders described herein certain nitro and/or halogen aromatic compounds such as are described in Patents Nos. 2,500,208 and 2,500,209. These compounds may be added to the coal-derived bitumen prior to the removal of the undissolvable matter therefrom in accordance with techniques described herein provided that the following operating temperature's do not exceed the temperature at which the compound reacts with the bitumen.

Alternatively, nitro or halogen aromatic compounds may be added to the binder subsequent to removal of undissolvable matter therefrom to produce a liquefiable single-phase material. Alternatively, the aforementioned compounds may be added to the binder during the mixing operation whereby the binder and carbon particles are mixed at a temperature of about 150° C. These compounds may be advantageously incorporated into the binder of the present invention in amounts up to about 45% by weight of the binder when such compounds are utilized to increase the coke residue of the binder. When the main object of the addition of such compounds is to take advantage of their lubricating qualities, the amount added to the binder is between about 2 and about 5% by weight, further provided that a portion of the added compound remains insoluble in the binder itself during the mixing operation.

In producing a binder or impregnating agent for electrodes in accordance with the present invention, it is desirable that the composition have between about 15 and 50% by weight of benzene-insoluble material (Barrett test No. B7) which, however, will be soluble or dissolvable in the binder itself. Small quantities of certain components of these binders may precipitate therefrom upon prolonged standing at room temperature, but these may readily be dissolved in the binder by heating or will become dissolved at temperatures employed during the mixing operation wherein the binder and carbon particles are admixed prior to the formation of "green" electrodes.

It has been found that graphite electrodes produced from a carbon aggregate and the present novel binders have improvements in electrical resistivities of 10% or more in comparison to graphite electrodes produced using the conventional coal tar pitch binders. It should be emphasized that the lowering of resistivity values in graphite electrodes even to a minor degree is particularly desirable and advantageous to the users of such electrodes. One of the main coats in operating an electrothermal or electrometallurgical high temperature furnace is the electric power consumption and the 10% or more reduction in electrical resistivity of my graphite electrodes is therefore highly desirable.

To more fully illustrate the nature and character of the invention but with no intention of being limited thereby, the following examples are set forth:

#### Example I

One hundred parts by weight of a commercial coal tar which contains about 14 to 15% of filterable solid phase material (undissolvable upon heating the tar to a temperature of 300° C.) was diluted with about 20 parts by weight of a high boiling coal tar distillate (boiling range 230° to 310° C., specific gravity 1.0-1.04). This mixture was heated to a temperature of about 200° C. To the liquefied material was added about 1% by weight of a high flow rate diatomaceous earth filter aid and the resulting mixture was filtered through a filter press containing a pre-coat of diatomaceous earth filter aid. The resulting filtrate was then heated to recover the solvent and heating was further continued at a temperature between about 400° to 500° C. until the material had a softening point of 86° C. (ball and ring). This material was substantially free from undissolvable matter and had a benzene-insoluble content of about 24%. It was used in the preparation of graphite electrodes as follows:

A calcined petroleum coke flour consisting of 50±2% of 48/200 mesh and the remainder minus 200 mesh was employed as the carbon aggregate. To 100 parts by weight of flour was admixed 36 parts by weight of the binder prepared in the above described manner and the mixing operation was conducted at about 160° C. The resulting mass was extruded through a die at a pressure of about 5,000 pounds per square inch at a temperature of about 90° to form a "green" electrode. The latter was baked to a temperature of 1,000° C. and then graphitized to a temperature of 2900° C. The resulting electrode had a longitudinal electrical resistivity ohms/in.<sup>3</sup> of  $29.2 \times 10^{-5}$ .

A graphite electrode prepared according to the above described process from petroleum coke flour and a commercially available coal tar pitch having a softening point of 85° C. and a benzene insoluble content of 23.5% had an electrical resistivity value of  $33.8 \times 10^{-5}$ . It can be seen that a 13.6% reduction or improvement in electrical resistivity is obtainable by employing the carbonaceous binders of the present invention as compared to electrodes produced from standard coal tar pitch binders.

#### Example II

A binder was prepared from another commercial coal tar as described in Example I, but the final heating operation was conducted to a point where the binder had a softening point of

109° C. and a benzene insoluble content of 28.5% by weight. When liquefied, the binder was substantially free from an insoluble phase.

An electrode mix was prepared by adding 36 parts by weight of this binder to 100 parts of calcined petroleum coke flour of the type employed in Example I and a graphite electrode was prepared as described in Example I. This electrode had an electrical resistivity value of  $28.2 \times 10^{-5}$  ohms/in.<sup>3</sup> which is a 16.5% reduction of improvement in resistivity compared to graphite electrodes prepared with conventional coal tar pitch binders.

*Example III*

An electrode was prepared from calcined petroleum coke employing 60 parts by weight of coke particles having a particle size distribution of 1 to 1 to 1 of 8-10: 10-14: 14-20 mesh, and 40 parts of coke flour of the type employed in Example I. To 100 parts by weight of this mixture was added 27 parts by weight of a coal tar-derived binder prepared as described in Example I. A mixing operation was conducted at about 160° C. A graphite electrode formed from this mixture in accordance with the procedure of Example I had electrical resistivity value of  $40 \times 10^{-5}$  ohms/in.<sup>3</sup>

To 100 parts by weight of the calcined petroleum coke mixture described above were added 27 parts by weight of a conventional coal tar pitch binder. Mixing was conducted at a temperature of about 160° C. and a graphite electrode was prepared from the resulting mixture in accordance with the procedure described in Example I. This electrode had an electrical resistivity of  $47.9 \times 10^{-5}$  ohms/in.<sup>3</sup> which is 19.7% higher than the electrode prepared with the novel binder used above.

*Example IV*

One hundred parts by weight of a commercial coal tar pitch (20% filterable solid phase) was heated to a temperature of 160° C. and diluted with 200 parts by weight of a high boiling coal tar distillate. After heating the mixture to about 200° C. it was centrifuged to concentrate the insoluble phase. The substantially solid-free soluble phase was heated to remove the solvent and heating was further continued at a temperature between 400 to 500° C. until the resulting material had a softening point of 95° C. This material had a benzene-insoluble content of 23% by weight and was free from undissolvable material (material which would not dissolve upon heating the binder to 250° C.).

A graphite electrode was prepared according to the procedure of Example II, and a similar improvement respecting electrical resistivity was observed.

While the foregoing examples particularly illustrate the use of coal tars and pitches as the source of the carbonaceous binders of the present invention and describe the preparation of said binders by particular types of filtration operation, it is to be understood that other compositions of the type herein described and which are within the scope of the expression "high boiling coal-derived liquefiable bitumens" may be employed without departing from the spirit of the invention. Furthermore, it is to be understood that other types of operations for the removal of the matter undissolvable in such compositions at temperatures below their coking temperatures may be employed providing such operations re-

tain substantial amounts of benzene-insoluble material in the resulting binders.

I claim as my invention:

5 1. A composition suitable as a binder for carbon particles and as an impregnant in the manufacture of graphite electrodes comprising essentially coal tar pitch substantially free from matter insoluble therein at a temperature between about 100° and about 400° C., said composition containing between about 15 and about 50% by weight of benzene-insoluble matter which is soluble therein and having a softening point of between about 85° and about 125° C.

15 2. A process for producing a composition suitable as a binder for carbon particles and as an impregnant in the manufacture of graphite electrodes from coal tar which contains matter substantially insoluble therein at a temperature between about 100° and about 400° C. which comprises filtering said tar in conjunction with a filter aid at a temperature between about 150° and 400° C. to produce a filtrate substantially free from undissolvable matter and heating the resulting filtrate to a temperature between about 25 400° and 525° C. until the material has a softening point between about 85° and about 125° C. and contains between about 15 and about 50% by weight of benzene-insoluble matter which is soluble in said material.

30 3. A process according to claim 2, wherein a high boiling aromatic diluent having a boiling range between about 200° and about 400° C. is added to the tar prior to filtration in an amount between about 20 and about 100 parts by weight of said diluent per 100 parts by weight of tar, said diluent being a solvent for the benzene-insoluble tar fraction but a non-solvent for said undissolvable matter.

40 4. A process for producing a composition suitable as a binder for carbon particles and as an impregnant in the manufacture of graphite electrodes from coal tar pitch which contains matter substantially insoluble therein at a temperature between about 100° and about 400° C., which comprises filtering said pitch in conjunction with a filter aid at a temperature between about 200° and about 400° C. to produce a filtrate substantially free from insoluble matter but which contains between about 15 and about 50% by weight 45 of benzene-insoluble matter which is soluble in said filtrate.

50 5. A process according to claim 4 wherein a high boiling aromatic diluent having a boiling range between about 200° and about 400° C. is added to the pitch prior to filtration in an amount between about 1 to about 5 parts by weight of solvent to 1 part by weight of pitch, said diluent being a solvent for the benzene-insoluble pitch fraction but a non-solvent for said undissolvable matter.

References Cited in the file of this patent

UNITED STATES PATENTS

| Number       | Name                   | Date           |
|--------------|------------------------|----------------|
| 951,993      | Lowry et al. -----     | Mar. 15, 1910  |
| 1,355,099    | Weiss -----            | Oct. 5, 1920   |
| 1,708,602    | Black et al. -----     | Apr. 9, 1929   |
| 70 2,024,106 | Levin -----            | Dec. 10, 1935  |
| 2,297,455    | Brautigam et al. ----- | Sept. 29, 1942 |
| 2,340,847    | Parker -----           | Feb. 1, 1944   |
| 2,395,853    | Fair -----             | Mar. 5, 1946   |
| 2,549,298    | Donigan -----          | Apr. 17, 1951  |